

M. A. ROSS.  
METHOD OF MANUFACTURING PLATE GLASS DEVICES.  
APPLICATION FILED JULY 31, 1912.  
1,075,794.

Patented Oct. 14, 1913

2 SHEETS—SHEET 1.

Fig. 1



Fig. 2



Witnesses:

Wm. Geiger  
A. Munday

Inventor:  
Myron A. Ross  
By Munday, Geiger, Udeort & Clarke,

Atlys.

M. A. ROSS.  
METHOD OF MANUFACTURING PLATE GLASS DEVICES.  
1,075,794.

APPLICATION FILED JULY 31, 1912.

Patented Oct. 14, 1913.

2 SHEETS—SHEET 2.

Fig. 4



Fig. 5



Witnesses:

Wm. Geiger  
J. M. Murphy.

Inventor:  
Myron A. Ross

By Munday, Evans, Adeock & Clarke,

Attest,

# UNITED STATES PATENT OFFICE.

MYRON A. ROSS, OF MORGANTOWN, WEST VIRGINIA, ASSIGNOR TO PRESSED PRISM PLATE GLASS COMPANY, OF MORGANTOWN, WEST VIRGINIA, A CORPORATION OF WEST VIRGINIA.

## METHOD OF MANUFACTURING PLATE-GLASS DEVICES.

1,075,794.

Specification of Letters Patent.

Patented Oct. 14, 1913.

Application filed July 31, 1912. Serial No. 712,447.

To all whom it may concern:

Be it known that I, MYRON A. ROSS, a citizen of the United States, residing in Morgantown, in the county of Monongalia 5 and State of West Virginia, have invented a new and useful Improvement in Methods of Manufacturing Plate-Glass Devices, of which the following is a specification.

This invention relates to improvements in 10 method of manufacturing plate glass devices.

An object of the invention is to provide a method or process for manufacturing plate glass devices, particularly of large size, such 15 as are adapted for illuminated, display, changeable sign use, and in which the letter, numeral, emblem or other symbol is formed with sharp, clear outlines and integrally with the plate, the entire glass-mass being 20 substantially homogeneous throughout.

Another object of the invention is to provide a method or process of manufacturing plate glass devices having the entire glass-mass homogeneous throughout and having 25 the letter, numeral, emblem or other symbol in protuberant relief, relatively thick as compared to the thickness of the plate, the raised portion, *per se*, being preferably one and one half, or even more, times as thick as 30 the plate, and in which the symbol in some instances is made lens-form, and forms with the plate a substantially plano-convex lens adapted to disperse and distribute light rays 35 passing through the glass, the portions in relief being preferably fluted longitudinally to thereby subdivide the larger lens into a plurality of smaller lenses in order that the shaft of light, as it emerges or is reflected from the plate glass device, may be given 40 substantial width.

A further object of the invention is to provide a method or process of manufacturing plate glass devices, in which the letter, numeral, emblem or other symbol is formed 45 wholly within, and has all portions removed from, the edges of the plate.

The invention furthermore consists in the 50 improvements in the steps and in the novel combination of the steps of the process as more fully disclosed hereinafter and set forth in the claim.

I am aware that it has been customary hitherto to form letters and numerals on

blocks by placing a gathering of glass in a mold and bringing a plunger down upon it, but it has been found that this method of manufacture is not practicable for making such articles of large size, the articles being limited generally to not more than three or four inches square. The finished article, even when the best results are obtained by this ordinary process of molding, lacks strength, is apt to be cracked, and when cut will break upon irregular lines, due to the inherent strains caused by the pressing step. I am aware, also, of a method of manufacturing prism glass by a process involving the two operations of first forming a sheet of glass, and secondly exerting pressure in a direction transverse to the plane of the sheet to form a plurality of prisms, regularly arranged over the entire surface of the sheet, as illustrated for instance in the patent to Ripley *et al.* No. 661,025, issued October 30th, 1900. In carrying out the process disclosed in this patent after the glass plate or sheet has been formed, the same is placed between a platen and a die, the latter having a plurality of closely arranged, equally spaced, parallel ribs, which results in producing an article having a regular or conventional design. Prism glass has also been made by the Ripley *et al.* process, having the ribs, ridges or prisms arranged both longitudinally and transversely of the plate in a conventional manner. But in all such instances, the glass plate is subjected substantially uniformly throughout its entirety to regularly distributed and equalized stresses and variations of temperature, the quantity of the glass-mass which goes to make up each rib or prism is comparatively small, each portion is only slightly displaced from its original position in the plate, and furthermore, the movement of the portion displaced is in paths practically uniform throughout, and without the thickness of the plate being greatly diminished.

In manufacturing plate glass devices having protuberant letters, numerals, emblems or other symbols, the predominant characteristics of which are their irregularity and diversity of outline and arrangement, it is necessary to displace some portions of the glass-mass relatively great distances and other portions only short distances, in di-

verse paths all substantially convergent toward and into the protuberant symbol being formed, and the quantity of the glass-mass required at one point is, in some instances, several times more than that required at another point, yet throughout all this irregular and uneven displacement, both as regards quantity and movement, and uneven variations of temperature and stresses at different portions of the plate, the chemical and physical homogeneity of the entire mass of glass composing the plate and symbol must be substantially preserved. This result I accomplish by my process described herein.

In my process I first form a sheet or plate of glass preferably by placing a gathering of glass on a platen and reducing it to plate-form in a state of what I term homogeneous consistency and molecular arrangement, as by a rolling or equivalent operation. In practice this is preferably done by rolling the glass while freely plastic, in the well known manner, and then while the plate is on a platen,—which may or may not be the platen upon which the gathering is rolled,—apply pressure in a direction transverse to the plate on portions located outside of the periphery of the letter or other symbol formed on the plate, and thus decrease the thickness of the plate at the portions where the pressure is applied, and cause portions of the glass-mass to flow toward the center or part of the plate where the letter or other symbol is located, the flow of the glass-mass taking place in paths substantially paralleling the surface of the plate and convergent toward the part where the letter or other symbol is formed, so that portions of the glass-mass are then forced up into and completely fill a deep recess in a die corresponding to the letter or other symbol desired. During this operation the edges of the plate may be confined as found desirable. In practice they are or may be self-confined by the less viscosity of the sheet at or near its somewhat cooler outer edges, which impedes the outward flow of the glass and causes it to flow inward and into the recess of the die. The plate with the letter or other symbol formed integrally therewith is then allowed to chill slightly to cause it to set sufficiently to be able to retain its shape, after which the plate glass device is annealed in the ordinary manner. In practising my invention, I may make the plate comparatively thin and the symbols, formed integrally therewith, relatively thick, and the height of the letters, numerals or other symbols may range from about eight to eighteen inches, and may be made even higher. If desired, the number of letters, numerals or other symbols on a single plate may be increased or multiplied so as to form, for instance, a complete word,

such as the word "Drugs", or any common stock sign-word or a series of numerals, the size and characteristics of the finished article being limited only by the size of the rolled plate on which the symbols are formed, which can, in actual practice, be made as large as sixty by ninety-six inches, the finished plate having a thickness of approximately five-sixteenths of an inch, and the solid symbols being approximately a further one-half inch in thickness.

In the drawing forming a part of this specification, Figure 1 is a plan view of a plate glass device, made by my process. Fig. 2 is a side elevation of the device shown in Fig. 1. Fig. 3 is an enlarged, detail, sectional view, approximately full size, and taken substantially on the line 3—3 of Fig. 1. Fig. 4 is a plan view of the plate or sheet showing thereon, in outline only, a letter such as is adapted to be made by my process, and illustrating, by means of arrows, the direction of flow of portions of the glass-mass, and Fig. 5 is a sectional view, taken on the line 5—5 of Fig. 4, showing, in dotted lines, the original thickness of the plate before the pressing operation takes place, and also indicating, by arrows, the paths followed by portions of the glass-mass during the pressing operation.

In the drawing, 10 denotes a rolled, rectangular plate having a plane back surface and which, as shown, is provided with a single, raised, solid symbol 11, formed integrally with the plate, the glass-mass of both members being substantially homogeneous throughout. The particular symbol shown in the drawing is the letter "F", but, as will be understood, other letters of the alphabet, punctuation marks, numerals, emblems or other symbols could be formed without departing from the spirit of the invention. Each portion of the raised symbol 11 is substantially lens-form, and is provided with a plurality of convex flutes or ribs 12 arranged longitudinally of each portion of the symbol.

The plate shown in the drawing is provided with only a single letter, and is adapted to be used in combination with a number of other plates similarly provided with letters for use in making up illuminated display signs, the letters of which are approximately one foot in height, although, as will be obvious, a single plate may be made with a plurality of letters or other symbols formed thereon, if desired.

After the plate or sheet is formed, pressure is applied to the same at portions surrounding the outline of the letter or other symbol being formed and at all such portions simultaneously, if desired, which will cause portions of the glass-mass to flow in diverse, substantially converging paths, as indicated by the arrows *a*, *a* in Fig. 4. In

doing this a die having a recess cut therein on its lower face, corresponding to the letter or other symbol desired to be formed, is placed over the plate and as the pressure is continued on the portions of the plate surrounding the symbol, the thickness of the plate will be diminished, as shown in Fig. 5, and displaced portions of the glass-mass will be caused to flow in the paths, as indicated by the arrows  $b, b$ , up into and to fill the recess in the die corresponding to the symbol, it being apparent that the quantity of glass displaced from the portions of the plate surrounding the symbol will approximate the quantity of glass required to fill the recess in the die to form the symbol. After the squeezing or pressing operation, the entire glass-mass is allowed to cool a sufficient time,—generally two or three seconds,—to cause the glass-mass to set, so that it may be properly handled and transferred to the annealing ovens without becoming distorted.

I claim:—  
25 The herein described process of making

figured glass sheets, which consists in first reducing a body of fluid glass to homogeneous consistency and molecular arrangement, in substantially the form of plate glass; then while the sheet is still plastic, forming a protuberant symbol upon one surface of the sheet and integral and homogeneous therewith, by reducing the thickness of the sheet and causing the glass of the body of the same to flow, for various distances and in various amounts as may be required by the irregular configuration of the symbol, in convergent directions and ultimately out from the surface of the sheet to form such symbol; and at the same time forming around the symbol an area of sheet glass of substantially uniform thickness; substantially as specified.

In testimony whereof, I have hereunto set my hand in the presence of two subscribing witnesses.

MYRON A. ROSS.

Witnesses:

HENRY LOVE CLARKE,  
JOSEPH HARRIS.